

## UNITED STATES PATENT OFFICE

2,171,781

## LUBRICATING OIL

Robert C. Cantelo, Whiting, Ind., assignor to  
 Sinclair Refining Company, New York, N. Y.,  
 a corporation of Maine

No Drawing. Application September 15, 1937,  
 Serial No. 163,916

7 Claims. (Cl. 87—9)

This invention relates to the treatment of hydrocarbon oils and, more particularly to the incorporation in hydrocarbon lubricating oils of certain compounds which have the effect of improving the physical characteristics and lubricating properties of the oils.

Hydrocarbon lubricating oils have a tendency to deteriorate upon standing for a reasonable length of time under ordinary storage conditions. 10 This tendency becomes greatly exaggerated under conditions of use, particularly where the oil is maintained at an elevated temperature for a considerable period of time. For instance, when used for lubricating internal combustion engines, such as employed in modern automobiles and aeroplanes where the oil is in contact with the rapidly moving and highly heated engine parts, this deterioration becomes pronounced and results in serious changes in the composition and 20 characteristics of the oil.

One of the consequences of this deterioration is the formation in the oil of a heavy sludge which collects after a time in the oil pump and oil lines of the engine, eventually clogging them to 25 such an extent as to prevent or greatly impair the efficient lubrication of the engine. This sludge-like material also becomes deposited on the pistons of the engine and frequently causes sticking of the piston rings and valves of the engine.

This deterioration further causes an increase in the viscosity of the lubricating oil, thereby putting a correspondingly increased load on the engine. Such increase in the viscosity over that 35 ordinarily selected for the conditions of use is particularly objectionable, for example, when starting the motor in cold weather.

It has also been found desirable to lower the pour point of hydrocarbon lubricating oils. Such 40 lubricating oils frequently have pour points in the neighborhood of 20° F. or even considerably higher, and the viscosity at low temperatures of such oils used as a lubricant is particularly objectionable when starting an internal combustion engine in cold weather.

Extensive research has been carried out in developing lubricating oils which are stable under conditions of storage and use and which have a pour point as low as possible. This work has 45 led to the addition to lubricating oils of certain materials thought to have a stabilizing influence on the oils by retarding the above-mentioned deterioration. Other materials have been added to these oils to lower the pour point thereof.

50 My invention provides a new type of compound

to be added to lubricating oils or the like whereby the objectionable deterioration of the oil is materially diminished, the viscosity and other physical characteristics of the oils are improved, and the pour point of the oil is advantageously 5 lowered. My invention also provides an improved lubricating oil in which the rate of sludge or gum formation is materially decreased and which has a substantially lowered pour point.

The formation of sludge in ordinary lubricating oils and the increase in viscosity under the conditions of use are generally recognized phenomena. The extent to which these phenomena occur, under uniform conditions, varies with the particular lubricating oil used, and the 15 rate at which they proceed in a particular oil generally increases as the temperature increases.

Special methods have been devised for measuring the rate of sludge-formation in various oils and under various temperature conditions. A 20 generally satisfactory method has been described in the American Society of Testing Materials Proceedings, vol. 24, page 967 whereby the time is determined in which 10 milligrams of sludge is formed in 10 grams of the oil maintained at a 25 definite temperature while air is bubbled through the oil at a specified rate. This time is designated "sludging time" and is a measure of the rate of sludge-formation in that particular oil under the particular conditions of the test. The 30 term "sludging time" as used hereinafter refers to the above-determined measure of the rate of sludge-formation and is a relative measure of the tendency of the oil to form sludge under conditions of storage or use.

I have discovered that the sludging time of hydrocarbon lubricating oils is greatly increased by the addition to the oil of a small proportion of a compound derived from erucic acid. In addition to increasing the sludging time, these 40 derivatives of erucic acid have a general effect of raising the viscosity index of the oil and appreciably lowering the pour point of the oil. Metallic and aromatic derivatives of erucic acid have been found to have these effects upon hydrocarbon lubricating oils when used in varying proportions. The metallic derivatives of erucic acid appear to be more effective, however, than the aromatic derivatives. Aluminum erucate, for example, has been found to be especially effective 50 although alpha naphthyl erucate and benzyl erucate may be used with particular advantage.

The derivatives of erucic acid used in accordance with my invention may be prepared, for example, by forming the sodium salt of erucic 55

acid and subjecting the salt to the action of a metallic salt capable of precipitating the desired metallic derivative of erucic acid or to the action of an aromatic compound, such as an alcohol, capable of reacting with erucic acid to give the desired derivative. The erucic acid is readily obtainable as the chief constituent of rapeseed oil.

In preparing a small quantity of the erucic acid, I used a blown rapeseed oil which had an acid number of 7.35, a saponification number of 203.0, an iodine value of 61.1, and an A. P. I. gravity of 15.2°. 3000 c. c. of this rapeseed oil were saponified by adding thereto a solution comprising 540 grams of sodium hydroxide dissolved in about 3000 c. c. of water. After complete saponification of the oil the mixture was diluted with five times its own volume of water and heated until all of the soap was in solution. A quantity of 36% hydrochloric acid was then added to the soap solution until no further precipitation occurred. The mixture was allowed to settle for about one hour and the aqueous layer then drawn off. The remaining oil layer was washed twice with water at a temperature of about 140° F. and the water drawn off after each of these washings. The oil layer which had been washed was dissolved in approximately three times its volume of 95% ethyl alcohol. Upon chilling the solution to a temperature of about -5 to 0° C. and maintaining the solution at this temperature for about five to six hours, crude erucic acid was precipitated from the solution. This crude erucic acid was separated from the solution by filtering and was then recrystallized twice by dissolving it in two parts by weight of 95% alcohol and by chilling the solution to a temperature between approximately -5 to 0° C. for each recrystallization. After recrystallizing the acid for the third time by dissolving it in one part of warm 95% alcohol and allowing the acid to crystallize from the solution at room temperature, a further yield of erucic acid was obtained from the filtrate of this third recrystallization by chilling the filtrate to a temperature of about -5 to 0° C. After removing by evaporation the alcohol held in the solid product separated during the three recrystallization operations together with that crystallized from the filtrate of the third recrystallization, a total yield of 470 grams of erucic acid was obtained.

Aluminum erucate was prepared from the erucic acid thus obtained by neutralizing 50 grams of the erucic acid with the theoretical quantity of sodium hydroxide in the form of 20° Bé. solution. 400 c. c. of a solution made up of one part of 95% alcohol and one part of water were added to the sodium hydroxide solution of the erucic acid, and this mixture was heated until all of the sodium erucate had completely dissolved. A solution comprising 17% by weight of aluminum sulphate was then added to the sodium erucate solution in an amount equivalent to 110% of the theoretical quantity of aluminum sulphate required to completely react with the sodium erucate. Aluminum erucate was coagulated by heating this mixture. After separating the precipitated aluminum erucate from the aqueous solution by decantation, the aluminum erucate was washed several times with water accompanied by decantation of the wash water from the solid product after each washing. Upon drying the product on a hot plate a yield was obtained which amounted to 80% of the theoretical yield of aluminum erucate.

The addition agents of my invention which are added to a hydrocarbon lubricating oil may comprise either a substantially pure salt of the erucic acid or it may comprise with advantage the salt of this erucic acid together with a small proportion of free erucic acid. For example, aluminum erucate precipitated from 100% neutralized erucic acid may be used as the addition agent, or the aluminum salt of a 90% neutralized erucic acid may be used with advantage. Moreover, the addition agent may comprise the substantially pure aluminum erucate to which a relatively small proportion of free erucic acid has been added. The presence or absence, as the case may be, of the free erucic acid in the addition agent had a distinct effect upon the modification of the physical characteristics of the oil by the addition agent.

My invention will be further described with specific reference to aluminum erucate. It is to be understood, however, that the following specific examples are merely illustrative of my invention as applied to particular oils and that my invention is not limited to the use of aluminum erucate or the following specific proportions thereof. Tables I and II show the effect of varying proportions of aluminum erucate on the viscosity, sludging time and pour point of a Pennsylvania motor oil having a gravity of 28.5, a flash point of 430° F., and a viscosity index of 100.1. The addition agent in Table I comprises aluminum erucate containing substantially no free acid. The addition agent in Table II comprises 90 parts of the aluminum erucate of Table I and 10 parts of erucic acid. The addition agent of Table II thus contains some free erucic acid.

Table I

| Percent addition agent in blend | 0     | 0.5   | 1.0   | 1.5   | 2.0   | 3.0   |
|---------------------------------|-------|-------|-------|-------|-------|-------|
| Vis. at 100° F.                 | 413   | 414   | 430   | 433   | 457   | 1465  |
| Vis. at 210° F.                 | 59.3  | 59.9  | 61.1  | 61.9  | 64.0  | 149.7 |
| V. I.                           | 100.1 | 102.4 | 103.4 | 106.6 | 108.9 | 122   |
| Sludging time (0.1% tar) hours  | 58    | 60    | 62    | 72    | 77    | 102   |
| Pour, ° F.                      | 5     | -10   | B-10  | B-10  | B-10  | B-10  |

Table II

| Percent addition agent in blend | 0     | 0.5   | 1.0   | 1.5   | 2.0   | 3.0   |
|---------------------------------|-------|-------|-------|-------|-------|-------|
| Vis. at 100° F.                 | 413   | 415   | 421   | 425   | 424   | 456   |
| Vis. at 210° F.                 | 59.3  | 59.9  | 60.5  | 60.7  | 60.6  | 62.7  |
| V. I.                           | 100.1 | 102.6 | 103.4 | 103.5 | 103.3 | 104.1 |
| Sludging time (0.1% tar) hours  | 58    | 23    | 54    | 82    | 84    | 125   |
| Pour, ° F.                      | 5     | 0     | -15   | -15   | -15   | -15   |

A consideration of the results shown in Tables I and II indicates that for this particular Pennsylvania motor oil the sludging time of blends of aluminum erucate in the oil is substantially independent of the amount of free erucic acid, up to at least 10%, in the addition agent. The sludging time and viscosity index are both markedly increased by the addition of the oil of 3% of aluminum erucate, regardless of the amount of free erucic acid, up to at least 10%, in the addition agent. The pour point of this Pennsylvania oil is lowered 15 to 20° F. by the addition of aluminum erucate over a wide range of percentages of aluminum erucate in the blend.

Tables III and IV show the effect of adding aluminum erucate to a hydrocarbon lubricating oil having a gravity of 20.8, a flash point of 370° F.,

a viscosity index of 23.4, and a pour point of  $-5^{\circ}$  F. The addition agent used in Table III is the same as that used in Table I, while the addition agent used in Table IV is the same as that used in Table II.

Table III

| Percent addition agent in blend       | 0    | 0.5  | 1.0  | 1.5  | 2.0  | 3.0   |
|---------------------------------------|------|------|------|------|------|-------|
| Vis. at $100^{\circ}$ F.              | 502  | 510  | 519  | 545  | 551  | 1407  |
| Vis. at $210^{\circ}$ F.              | 53.9 | 54.0 | 54.7 | 55.7 | 56.5 | 122.4 |
| V. I.                                 | 23.4 | 21.3 | 26.3 | 31.9 | 34.9 | 112   |
| Sludging time (0.1 percent tar) hours | 8.5  | 9    | 17.5 | 20.5 | 21.5 | 27.5  |

Table IV

| Percent addition agent in blend       | 0    | 0.5  | 1.0  | 1.5  | 2.0  | 3.0  |
|---------------------------------------|------|------|------|------|------|------|
| Vis. at $100^{\circ}$ F.              | 502  | 506  | 502  | 502  | 508  | 552  |
| Vis. at $210^{\circ}$ F.              | 53.9 | 53.6 | 53.5 | 53.7 | 54.3 | 56.4 |
| V. I.                                 | 23.4 | 17.5 | 17.8 | 24.9 | 25.9 | 32.3 |
| Sludging time (0.1 percent tar) hours | 8.5  | 9.5  | 14.0 | 21.0 | 18.0 | 30   |

The results of Tables III and IV indicate that for a hydrocarbon lubricating oil having the foregoing physical characteristics the addition of aluminum erucate to the oil increases the sludging time of the oil substantially independently of the amount of free erucic acid, up to at least 10%, in the addition agent. The viscosity index of the oil is also increased by the incorporation of aluminum erucate in the oil, this effect being more pronounced in the blends containing 3% aluminum erucate.

The aluminum erucate used to produce the results shown in Tables I through IV was prepared from an unblown rapeseed oil having a saponification number of 178, an acid number of 1.13, and an iodine value of 100. The erucic acid was prepared from this rapeseed oil in accordance with the method described by Noller and Talbot in *Organic Synthesis*, vol. X, p. 44 (John Wiley & Sons, Inc.). The erucic acid thus obtained had a saponification number of 148, an acid number of 132, and an iodine value of 63.1. This erucic acid was dissolved in the theoretical quantity of  $20^{\circ}$  Bé. aqueous sodium hydroxide solution, and aluminum erucate was precipitated from this solution by adding thereto an aqueous solution of aluminum sulphate containing an excess of aluminum sulphate over the theoretical quantity necessary for complete precipitation. The solid aluminum erucate was separated from the solution by filtration, and the solid product was washed with water and subsequently dried.

The effectiveness of aluminum erucate in lowering the pour point of lubricating oils is indicated in Table V which shows the results of the incorporation of small quantities of aluminum erucate in three distinct types of hydrocarbon lubricating oils. Blank oil "A" has a gravity of 28.4, a flash point of  $430^{\circ}$  F., a viscosity of 431 seconds Saybolt Universal at  $100^{\circ}$  F., a viscosity index of 103.4, and a pour point of  $5^{\circ}$  F. Blank oil "B" has a gravity of 27.7, a flash point of  $445^{\circ}$  F., a viscosity of 618 seconds Saybolt Universal at  $100^{\circ}$  F., a viscosity index of 103, and a pour point of  $20^{\circ}$  F. Blank oil "C" has a gravity of 26.4, a flash point of  $395^{\circ}$  F., a viscosity of 200 seconds Saybolt Universal at  $100^{\circ}$  F., a viscosity index of 73.0, and a pour point of  $10^{\circ}$  F.

Table V

| Percent addition agent | Blank "A" | Blank "B" | Blank "C" |
|------------------------|-----------|-----------|-----------|
| 0.25                   | -5        | 20        | B-15      |
| 0.50                   | -15       | 20        | B-15      |
| 0.75                   | -15       | 10        | B-15      |
| 1.0                    | -10       | 0         | -----     |
| 1.5                    | -5        | -5        | -----     |
| 2.0                    | 0         | -5        | -----     |

From the above tabulation it is apparent that the pour point of blank oil "A" is reduced to a minimum by the addition of about 0.5% aluminum erucate, that the pour point of blank oil "B" is reduced to a minimum by the addition of approximately 1.5% aluminum erucate, while the pour point of blank oil "C" is reduced to below  $-15^{\circ}$  F. by the incorporation therein of 0.25% aluminum erucate.

It must be emphasized, however, that my invention is not to be limited by the proportions of the addition agent used in the foregoing illustrations. For example, it has been found that as little as 0.1% of aluminum erucate has a salutary effect in lowering the pour point of certain hydrocarbon lubricating oils, while it has also been found that high percentages, that is, up to 10% of aluminum erucate has a favorable effect in reducing the tendency of hydrocarbon lubricating oils to form sludge under conditions of use. When percentages in the neighborhood of 5 to 10% of the addition agent are used, the addition agent may contain with advantage larger proportions than 10% of free erucic acid.

Thus, it will be seen from the foregoing tabulations that the incorporation in hydrocarbon lubricating oils of a small proportion of aluminum erucate for example, increases the sludging time of the oil, increases, in most instances, the viscosity index of the oil, and greatly reduces the pour point of the oil. The effectiveness of small quantities of this addition agent together with the fact that it may be readily prepared from a relatively inexpensive raw material imparts to this addition agent, and the others hereinbefore enumerated, a low cost and a high degree of efficiency.

I claim:

1. The method of inhibiting the formation of sludge in a hydrocarbon lubricating oil and of lowering the pour point thereof which comprises incorporating in the oil between about 0.5 and 3.0% of a metallic salt of erucic acid.

2. The method of inhibiting the formation of sludge in a hydrocarbon lubricating oil and of lowering the pour point thereof which comprises incorporating in the oil between about 0.5 and 3.0% of aluminum erucate.

3. The method of inhibiting the formation of sludge in a hydrocarbon lubricating oil and of lowering the pour point thereof which comprises incorporating in the oil between about 0.5 and 3.0% of aluminum erucate containing a relatively small proportion of free erucic acid.

4. An improved lubricating oil resistant to sludge formation and having a reduced pour point which comprises a hydrocarbon lubricating oil containing between about 0.5 and 3.0% by weight of a metallic salt of erucic acid.

5. An improved lubricating oil resistant to sludge formation and having a reduced pour point which comprises a hydrocarbon lubricating oil containing between about 0.5 and 3.0% by weight of a metallic salt of erucic acid together

with a relatively smaller proportion of free erucic acid.

6. An improved lubricating oil resistant to sludge formation and having a reduced pour point which comprises a hydrocarbon lubricating oil containing between about 0.5 and 3.0% by weight aluminum erucate.

7. An improved lubricating oil resistant to sludge formation and having a reduced pour point which comprises a hydrocarbon lubricating oil containing between about 0.5 and 3.0% aluminum erucate together with a relatively smaller proportion of free erucic acid.

ROBERT C. CANTELO.